# EUROPEAN PATENT SPECIFICATION

(11) **EP 0 997 317 B1**
(45) Date of publication and mention of the grant of the patent: **08.10.2003**
(21) Application number: 98203608.9
(22) Date of filing: 26.10.1998
(51) Int. Cl.: B41N 3/03

(54) **A lithographic base for use in non-impact printing**
Lithographischer Träger für anschlagloses Drucken
Support lithographique pour l'impression sans frappe

(43) Date of publication of application: 03.05.2000
(73) Proprietor: AGFA-GEVAERT, 2640 Mortsel (BE)
(72) Inventor: Verschueren, Eric Agfa-Gevaert N.V., 2640 Mortsel (BE)

(56) References cited:
- US-A- 2 805 621
- US-A- 2 941 466
- US-A- 3 230 873
- US-A- 4 046 946
- US-A- 4 851 150

## Description

### FIELD OF THE INVENTION.

The present invention relates to a lithographic base. More particularly the present invention relates to an hydrophilic lithographic surface layer with improved mechanical properties.

### BACKGROUND OF THE INVENTION.

Lithography is the process of printing from specially prepared surfaces, some areas of which are capable of accepting lithographic ink, whereas other areas, when moistened with water, will not accept the ink. The areas which accept ink form the printing image areas, generally hydrophobic areas, and the ink-rejecting areas form the background areas, generally hydrophilic areas.

In the art of photolithography, a photographic material is made imagewise receptive to oily or greasy inks in the photo-exposed (negative-working) or in the non-exposed areas (positive-working) on a hydrophilic background.

In the production of common lithographic printing plates, also called surface litho plates or planographic printing plates, a lithographic base that has affinity to water or obtains such affinity by chemical treatment is coated with a thin layer of a photosensitive composition. Compositions for that purpose include light-sensitive materials such as light-sensitive polymers, diazonium salts or resins, a photoconductive layer, a silver halide emulsion etc. These materials are then image-wise exposed to actinic radiation and processed in the appropriate manner so as to obtain a lithographic printing plate.

In another embodiment, a silver precipitating (nucleating) agent is located in or on top of the hydrophilic surface. An image is obtained on the precipitating layer according to the silver salt diffusion transfer process by contacting said precipitating layer with an exposed silver halide emulsion in the presence of a silver halide developing agent and a silver halide solvent.

According to another embodiment there is provided a heat mode imaging element for making a lithographic printing plate comprising on a lithographic base with a hydrophilic surface a first layer including a polymer, soluble in an aqueous alkaline solution and a top layer on the same side of the lithographic base as the first layer which top layer is IR-sensitive and unpenetrable for an alkaline developer wherein said first layer and said top layer may be one and the same layer.

A hydrophilic receiving layer can also be used for xerography, electrography, thermosublimation, thermal transfer and other image-forming techniques.

Several types of supports can be used for the manufacturing of a lithographic imaging printing plate. Common supports are for example organic resin supports, e.g.polyesters,and paper bases, e.g. polyolefin coated paper. These supports are first coated with a hydrophilic layer forming the hydrophilic lithographic background of the printing plate.

It is known to use as hydrophilic layer in these systems a layer containing polyvinyl alcohol and hydrolyzed tetra(m)ethyl orthosilicate and titanium dioxide and preferably also silicium dioxide as described in e.g. **GB-P- 1 419 512**, **FR-P- 2 300 354**, **US-P- 3 971 660** and **4 284 705, EP-A- 405 016** and **450 199.**

To obtain superior physical properties, it is very important to control the drying process. Avoiding drying stress results in materials with superior physical qualities. In fact, these drying stress, caused by the pressure gradient in the liquid phase, results in the occurance of microscopic fractures. The exterior of the gel shrinks much faster than the interior so that tensile stresses arise that tend to fracture the network at the exterior. These fractures propagate easily during the further drying process.

A number of measures can be taken to avoid these defects. To obtain good results, aging the gel before drying is recommended. However this is uneconomical and industrially not feasible.

### OBJECTS OF THE INVENTION

It is an object of the invention to provide a hydrophilic layer, for use in a printing system with excellent physical properties.

It is further an object of the present invention to provide a hydrophilic layer which can be coated economically.

Further objects of the present invention will become clear from the description hereinafter.

### SUMMARY OF THE INVENTION

According to the present invention there is provided a lithographic base comprising a support and a hydrophilic layer thereon containing a hydrophilic binder , TiO₂ particles and wherein said layer is cross-linked, characterized in that the total volume of pores of said lithographic base is more than 0.0007 cm³ /g.

### DETAILED DESCRIPTION OF THE INVENTION

Preferably the total volume of pores of said lithographic base is at least 0.0010 cm³ /g.

According to the present invention, the lithographic base having a hydrophilic surface comprises a flexible support, such as plastic film, provided with a cross-linked hydrophilic layer. A particularly suitable cross-linked hydrophilic layer may be obtained from a hydrophilic binder cross-linked with a cross-linking agent such as formaldehyde, glyoxal, polyisocyanate, zirconium compounds, titanates or a hydrolysed tetra-alkylorthosilicate. The latter is particularly preferred.

As hydrophilic binder there may be used hydrophilic (co)polymers or mixtures such as for example, homopolymers and copolymers of vinyl alcohol,polyvinyl pyrrolidone,starch or modified starch, acrylamide, methylol acrylamide, methylol methacrylamide, acrylate acid, methacrylate acid, hydroxyethyl acrylate, hydroxyethyl methacrylate or maleic anhydride/vinylmethylether copolymers. The hydrophilicity of the (co)polymer or (co)polymer mixture used is preferably the same as or higher than the hydrophilicity of polyvinyl acetate hydrolyzed to at least an extent of 60 percent by weight, preferably 80 percent by weight.

The amount of crosslinking agent, in particular of tetraalkyl orthosilicate, is preferably at least 0.2 parts by weight per part by weight of hydrophilic binder, more preferably between 0.5 and 5 parts by weight, most preferably between 0.8 parts by weight and 3 parts by weight.

A cross-linked hydrophilic layer in a lithographic base used in accordance with the present embodiment preferably also contains substances that increase the mechanical strength and the porosity of the layer. For this purpose colloidal silica may be used. The colloidal silica employed may be in the form of any commercially available water-dispersion of colloidal silica for example having an average particle size up to 40 nm, e.g. 20 nm.

A cross-linked hydrophilic layer in a lithographic base used in accordance with the present embodiment also contains in addition inert particles of larger size than the colloidal silica i.e. particles having an average diameter of at least 100 nm which are particles of titanium dioxide. By incorporating these particles the surface of the cross-linked hydrophilic layer is given a uniform rough texture consisting of microscopic hills and valleys, which serve as storage places for water in background areas. The amount of titanium dioxide is at least 55%, more preferably at least 62 % of the total amount of the hydrophilic layer.

The weight of a cross-linked hydrophilic layer in a lithographic base in accordance with this embodiment may vary in the range of 0.2 to 25 g/m² and is preferably 1 to 15 g/m².

As flexible support of a lithographic base in connection with the present embodiment paper or polyolefin paper can be used. It is particularly preferred to use a plastic film e.g. subbed polyethylene terephthalate film, subbed polyethylene naphthalate film, cellulose acetate film, polystyrene film, polycarbonate film etc... The plastic film support may be opaque or transparent.

It is particularly preferred to use a polyester film support to which an adhesion improving layer has been provided. Particularly suitable adhesion improving layers for use in accordance with the present invention comprise a hydrophilic binder and colloidal silica as disclosed in **EP-A-,619 524**, **EP-A- 620 502** and **EP-A- 619 525.** Preferably, the amount of silica in the adhesion improving layer is between 200 mg per m² and 750 mg per m². Further, the ratio of silica to hydrophilic binder is preferably more than 1 and the surface area of the colloidal silica is preferably at least 300 m² 5 per gram, more preferably at least 500 m² per gram.

The hydrophilic layer also contains drying control chemical additives.(DCCA's) As DCCA following classes of chemical compounds can be used:
- low molecular weight polyhydric alcohols such as ethylene glycol, diethylene glycol, triethylene glycol, tetraethylene glycol, dipropylene glycol, propylene glycol, pentane diol, glycerol, butane triol, trimethylolpropane, pentaerythritol, dipentaerythritol, 1-monoacetylglycerol and so on;
- liquid amides such as formamide, acetamide, propanamide and so on.

Said DCCA's can be used in combination and are preferably used in an amount between 100 and 1500 mg/m².

Solid acids should be excluded.

Said hydrophilic layer are suitable for heat mode imaging elements, ink jet printing, electrostatic printing, thermal transfer 1 printing, laser ablation transfer, thermal ablation transfer, laser transfer printing, electrographic printing, pen plotter, manual writing, xerographic printing, tonerjet printing.

### EXAMPLE 1 (Comparative example)

A 0.175 mm thick polyester foil was coated with a layer from a 23.6 % aqueous solution at pH 4, with a wet coating thickness of 50 µm. This layer was after chilling for 30 sec at 10°C dried at a temperature of 50°C with a moisture content of the air of 4 g/m³ for at least 3 minutes.

The resulting hydrophilic layer contained 8990 mg/m² TiO₂, 900 mg/m² SiO₂, 990 mg/m² polyvinylalcohol, 81.6 mg/m² SAPONIN ™, 36.8 mg/m² of HOSTAPON T ™ and 605 mg/m² of FT248 ™.

In advance to the preparation of the coating solution a dispersion was made comprising the above mentioned TiO₂, SiO₂ and polyvinylalcohol.

TiO₂ with average particle size between 0.3 and 0.5 µm was used. The used polyvinyl alcohol is hydrolyzed polyvinyl acetate, commercially available at Wacker Chemie GmbH, Germany under the trademark POLYVIOL WX ™. The SiO₂ mentioned above is added as a dispersion of hydrolyzed tetramethyl orthsilicate to the dispersion. SAPONIN is a nonionic surfactant mixture consisting of esters and polyglycosides, commercially available at Merck. HOSTAPON T is an anionic surfactant, commercially available at Hoechst AG. FT248 is an anionic perfluoro surfactant, commercially available at Bayer AG.

### EXAMPLE 2

The same composition was prepared in the same way as this described in example 1, with the exception that the hydrophilic layer comprised also 90.0 mg/m² of glycerol.

### EXAMPLE 3

The same composition was prepared in the same way as this described in example 1, with the exception that the hydrophilic layer comprised also 250.0 mg/m² of glycerol.

### EXAMPLE 4

The same composition was prepared in the same way as this described in example 1, with the exception that the hydrophilic layer comprised also 500.0 mg/m² of glycerol.

### EXAMPLE 5

The same composition was prepared in the same way as this described in example 1, with the exception that the hydrophilic layer comprised also 90.0 mg/m² of glycerol and 100 mg/m² of acetamide.

### EXAMPLE 6

The same composition was prepared in the same way as this described in example 1, with the exception that the hydrophilic layer comprised also 90.0 mg/m² of glycerol and 200 mg/m² of acetamide.

### EXAMPLE 7

The same composition was prepared in the same way as this described in example 1, with the exception that the hydrophilic layer comprised also 460.0 mg/m² of glycerol and 100 mg/m² of acetamide.

### EXAMPLE 8

The same composition was prepared in the same way as this described in example 1, with the exception that the hydrophilic layer comprised also 460.0 mg/m² of glycerol and 100 mg/m² of acetamide.

### EXAMPLE 9

The same composition was prepared in the same way as this described in example 1, with the exception that the hydrophilic layer comprised also 460.0 mg/m² of glycerol and 1000 mg/m² of acetamide.

### EXAMPLE 10

The same composition was prepared in the same way as this described in example 1, with the exception that the hydrophilic layer comprised also 90.0 mg/m² of glycerol and 560 mg/m² of oxalic acid.

### EXAMPLE 11

The same composition was prepared in the same way as this described in example 1, with the exception that the hydrophilic layer comprised also 90.0 mg/m² of glycerol and 1130 mg/m² of oxalic acid.

### Total pore volume of the lithographic base.

The total pore volume of the lithographic base was measured by a Micromeritics ASAP 2400 apparatus. Therefore, the material, including the support, was cut in little pieces and brought into the apparatus, then a sorption/desorption of the material was measured with nitrogen gas as adsorbate.

From the obtained sorption/desorption isotherm, the total pore volume was calculated by the method of Barett, Joyner and Hallender.

### Physical properties

The physical properties of the imaging element were evaluated by measuring the scratch resistance. In this test the mechanical properties and the adhesion of the coating to the support become clear.

### Scratching the hydrophilic layer.

The above mentioned materials in comparative example 1 and examples 2 till 11 were scratched in a standard test. First, swelling of the lithographic base in distilled water occured under equilibrium conditions. For safety, a time of 2 minutes was applied. In this test scratches were formed by displacing needles at a speed of 96 cm/min, under well defined loads. The needles were of type rubin with a radius of 1.5 mm. 15 scratches were formed under following loads: 57 - 85 - 114 - 142 - 170 - 113 - 169 - 225 - 282 - 338 - 400 - 600 - 800 - 1000 en 1200 mN.

### Evaluation of the scratch resistance of the hydrophilic layer.

The 15 scratches were controlled on width of damage and given a corresponding quotation as indicated in table 1.
When the depth of the scratch was unto the support, this means the total layer was removed, an extra value was summated. This phenomenon was visible by a discoloration from white to transparent on the scratch region. This value was 3 when the discoloration was locally. When the entire scratch was transparent a value of 5 was added.

**Table 1**

| Quotation | Width of scratch |
|---|---|
| 0 | no scratch visible |
| 0.5 | scratch smaller than 50µm |
| 1 | width between 50 and 100 µm |
| 2 | width between 100 and 150 µm |
| 3 | width between 150 and 200 µm |
| 4 | width greater than 200 µm |
| + 3 | when scratch is broken transparent line |
| + 5 | when scratch is fully transparent |

A summation of all given quotations resulted in the scratch resistance of te material. The lower the value, the better the scratch resistance.

### Results

| | Scratch resistance | Total pore volume in cm³ /g |
|---|---|---|
| Example 1 | 38 | 0.000101 |
| Example 2 | 11 | 0.000087 |
| Example 3 | 0 | 0.000768 |
| Example 4 | 0 | 0.001067 |
| Example 5 | 0 | 0.000790 |
| Example 6 | 0 | 0.001612 |
| Example 7 | 3 | 0.000912 |
| Example 8 | 0 | 0.001272 |
| Example 9 | 0 | 0.001872 |
| Example 10 | 31 | 0.000070 |
| Example 11 | 18 | 0.000079 |

It is clear from the results of table 2 that all the examples according to the invention have a very good to excellent scratch resistance, much better than the comparative example.

## Claims

1. A lithographic base comprising a support and a hydrophilic layer thereon containing a hydrophilic binder, TiO₂ particles and wherein said layer is cross-linked, **characterized in that** the total volume of pores of said lithographic base is more than 0.0007 cm³ /g.

2. A lithographic base according to claim 1 wherein the total volume of pores of said lithographic base is at least 0.0010 cm³ /g.

3. A lithographic base according to claim 1 or 2 wherein the hydrophilic layer comprises one or more drying control chemical additive(s).

4. A lithographic base according to claim 3 wherein the drying control chemical additive(s) comprise(s) (are)a low molecular weight polyhydric alcohol.

5. A lithographic base according to claim 4 wherein the drying control chemical additive(s) comprise(s) glycerol.

6. A lithographic base according to claim 3 wherein the drying control chemical additive(s) comprise(s) a liquid amide.

7. A lithographic base according to claim 6 wherein the liquid amide is acetamide.

8. A lithographic base according to any of claim 3 to 7 wherein the drying control chemical additive(s) is (are) present in an amount between 100 and 1500 mg/m².

9. A lithographic base according to any of claims 1 to 8 wherein the hydrophilic layer has a weight between 1 and 15 g/m².

10. A lithographic base according to any of claims 1 to 9 wherein the titanium oxide is used in an amount of at least 55% of the total amount of the hydrophilic layer.

## Patentansprüche

1. Eine lithografische Unterlage mit einem Träger und einer darüber vergossenen, hydrophilen, vernetzten, ein hydrophiles Bindemittel und TiO₂-Teilchen enthaltenden Schicht, **dadurch gekennzeichnet, daß** das Gesamtvolumen der Poren der lithografischen Unterlage mehr als 0,0007 cm³/g beträgt.

2. Lithografische Unterlage nach Anspruch 1, **dadurch gekennzeichnet, daß** das Gesamtvolumen der Poren der lithografischen Unterlage zumindest 0,0010 cm³/g beträgt.

3. Lithografische Unterlage nach Anspruch 1 oder 2, **dadurch gekennzeichnet, daß** die hydrophile Schicht eine oder mehrere die Trocknung steuernde chemische Additive enthält.

4. Lithografische Unterlage nach Anspruch 3, **dadurch gekennzeichnet, daß** das (die) chemische(n) Additiv(e) für die Steuerung der Trocknung einen niedermolekularen mehrwertigen Alkohol enthält (enthalten).

5. Lithografische Unterlage nach Anspruch 4, **dadurch gekennzeichnet, daß** das (die) chemische(n) Additiv(e) für die Steuerung der Trocknung Glycerin enthält (enthalten).

6. Lithografische Unterlage nach Anspruch 3, **dadurch gekennzeichnet, daß** das (die) chemische(n) Additiv(e) fürdie Steuerung der Trocknung ein flüssiges Amid enthält (enthalten).

7. Lithografische Unterlage nach Anspruch 6, **dadurch gekennzeichnet, daß** das flüssige Amid Acetamid ist.

8. Lithografische Unterlage nach einem der Ansprüche 3 bis 7,
**dadurch gekennzeichnet, daß** das (die) chemische(n) Additiv(e) für die Steuerung der Trocknung in einer Menge zwischen 100 und 1.500 mg/m² enthalten ist (sind).

9. Lithografische Unterlage nach einem der Ansprüche 1 bis 8,
**dadurch gekennzeichnet, daß** die hydrophile Schicht ein Gewicht zwischen 1 und 15 g/m² aufweist.

10. Lithografische Unterlage nach einem der Ansprüche 1 bis 9,
**dadurch gekennzeichnet, daß** das Titanoxid in einer Mindestmenge von 55%, bezogen auf die Gesamtmenge der hydrophilen Schicht, verwendet wird.

## Revendications

1. Base lithographique comprenant un support et une couche hydrophile sur ce dernier, contenant un liant hydrophile, des particules de dioxyde de titane, et dans laquelle ladite couche est réticulée, **caractérisée en ce que** le volume total des pores de ladite base lithographique est supérieur à 0,0007 cm³/g.

2. Base lithographique selon la revendication 1, dans laquelle le volume total des pores de ladite base lithographique s'élève à au moins 0,0010 cm³/g.

3. Base lithographique selon la revendication 1 ou 2, dans laquelle la couche hydrophile comprend un ou plusieurs additifs chimiques pour le réglage du séchage.

4. Base lithographique selon la revendication 3, dans laquelle les additifs chimiques de réglage du séchage comprennent un alcool polyvalent à bas poids moléculaire.

5. Base lithographique selon la revendication 4, dans laquelle les additifs chimiques de réglage du séchage comprennent du glycérol.

6. Base lithographique selon la revendication 3, dans laquelle les additifs chimiques de réglage du séchage comprennent un amide liquide.

7. Base lithographique selon la revendication 6, dans laquelle l'amide liquide est l'acétamide.

8. Base lithographique selon l'une quelconque des revendications 3 à 7, dans laquelle les additifs chimiques de réglage du séchage sont présents en une quantité entre 100 et 1500 mg/m².

9. Base lithographique selon l'une quelconque des revendications 1 à 8, dans laquelle la couche hydrophile possède un poids entre 1 et 15 g/m2

10. Base lithographique selon l'une quelconque des revendications 1 à 9, dans laquelle l'oxyde de titane est utilisé en une quantité qui représente au moins 55 % de la quantité totale de la couche hydrophile.
